

# UNITED STATES PATENT OFFICE.

JAMES RAMSEY SPEER, OF TRAPPE, MARYLAND.

## ALLOY OF IRON.

1,105,341.

Specification of Letters Patent. Patented July 28, 1914.

No Drawing.

Application filed February 24, 1914. Serial No. 820,566.

To all whom it may concern:

Be it known that I, JAMES RAMSEY SPEER, a citizen of the United States, residing at Trappe, in the county of Talbot and State of Maryland, have invented new and useful Improvements in Alloys of Iron, of which the following is a specification.

My invention, broadly stated, relates to alloys of iron containing a larger percentage of chromium than nickel. While I do not fix any definite percentage which the chromium must have over the nickel, I prefer that the nickel shall range from .25%–1% of the total alloy and that the chromium shall range from .5% to 1.5% thereof. I have obtained most excellent results by having the quantity of nickel in the neighborhood of 50% of the quantity of chromium, and generally speaking I prefer that these two elements have this relationship to each other. Specific analysis of castings herein-after set forth will illustrate some of the proportions of nickel and chromium wherein I regard the quantity of nickel as being in the neighborhood of 50% of the quantity of chromium, but these analyses are to be taken merely as illustrative, as the proportions of the nickel and chromium might be somewhat changed from the said analyses and still have the nickel in the neighborhood of 50% of the chromium. In the claims, the word, substantially, is to be understood to have the meaning of the phrase "in the neighborhood of," as above used.

In making castings from my alloy, the iron, chromium and nickel have been accompanied with silicon, sulfur, phosphorus, manganese, and carbon, but, in the broader aspects of my invention, my invention is not limited to any particular elements which accompany the iron, chromium and nickel. The elements above named may be accompanied with small quantities of copper, tungsten, and other ingredients which do not materially affect the character of the alloy as hereinafter described.

As is well known sulfur and phosphorus are ingredients of iron ore and cannot be wholly eliminated, at least, in the commercial manufacture of iron and steel. As I cannot prevent their presence in my product, I retain for my best products as small amounts of them as practicable with the methods employed for the manufacture of my alloy. Sulfur and phosphorus may be regarded as impurities which may be elimi-

nated in some cases so far as practicable with the mode of manufacture or retained in other cases to such a degree as not to make the articles undesirable for the purposes required.

I regard my invention as including cast iron alloys comprising the elements and substantially the percentages following: Silicon over .1% to 3%; chromium .5% to 1.5%; nickel .25% to 1%; sulfur over .05% to .2%; phosphorus over .12% to 1.5%; manganese over .45% to 1%; and total carbon 1% to 4%.

The control of the silicon and carbon is as essential as in usual foundry practice and these elements must vary in a wide range with the sections and weights of the castings.

I will give a few analyses showing the actual composition of articles made in accordance with my invention, the numerals indicating the percentages of the elements. These analyses are merely illustrative and do not limit me to the precise proportion of ingredients specified. These analyses are as follows:

| Sl.  | S.    | P.    | Mn. | Total C. | Ni. | Cr.  |    |
|------|-------|-------|-----|----------|-----|------|----|
| 1.75 | .098  | .129  | .64 | 3.52     | .65 | 1.17 | 85 |
| 1.55 | ..... | .166  | .64 | 3.55     | .56 | 1.00 |    |
| 2.08 | .064  | .169  | .62 | 3.50     | .58 | 1.06 |    |
| 1.70 | .100  | ..... | .59 | 3.52     | .62 | 1.13 |    |
| 1.86 | .093  | .153  | .61 | 3.56     | .60 | 1.15 |    |
| 1.85 | .080  | .170  | .66 | 3.56     | .58 | 1.10 |    |
| 1.52 | .108  | ..... | .70 | 3.62     | .54 | 1.06 |    |
| 1.88 | .105  | .122  | .58 | 3.55     | .54 | 1.08 | 90 |
| 1.92 | .094  | ..... | .67 | 3.58     | .52 | 1.06 |    |
| 1.25 | ..... | ..... | .55 | 3.92     | .52 | 1.08 |    |
| 1.51 | ..... | ..... | .62 | 3.58     | .56 | 1.18 |    |
| 1.63 | .087  | .184  | .66 | 3.52     | .45 | .98  |    |
| 1.75 | .103  | .167  | .65 | 3.55     | .58 | 1.25 |    |
| 1.95 | .090  | .123  | .66 | 3.55     | .52 | 1.18 |    |
| 1.81 | .090  | ..... | .64 | 3.48     | .55 | 1.25 | 95 |

The percentage of iron remains about the same in all cases for castings of similar sections and weights, and the aggregate total of the other elements remains about the same in all cases, and if the percentage of one or more of these elements is increased or diminished the others or some of them will be correspondingly decreased or increased within the limits of good manufacturing practice.

The articles made according to these analyses were hard and resistant to the action of abrasion or wear under heat. The life of my alloy is several times longer than the best grade of cast iron. I regard the amount of nickel in each of these analyses to be approximately or in the neighborhood of fifty

per cent. of the quantity of chromium. My alloy like cast iron may be cut and turned by machine tools. Under the acetylene torch, it is as resistant as cast iron, and in 5 its inability to show elasticity or elongation or reduction of area it resembles cast iron. It is more brittle than "adamite" which is the subject-matter of Letters Patent, No. 1,071,364 granted August 26, 1913, to myself 10 and William L. Forster. It is intermediate in quality between cast iron and adamite and is suitable for manufacturing the cheaper grades of rolling mill plugs and pipe balls, brake shoes, and various other 15 articles where abrasion and not high tensile strength determine the use and where precision of analysis to correspond to use is not so vital.

It is feasible, and probably for commercial 20 purposes most advisable, to produce my alloy in a cupola or like furnace.

When the sections of my alloy vary and are not uniform, it is advisable to anneal it to give it uniform strength and hardness. 25 In this feature, my alloy is very much like steel. Castings having large sections may be hardened in the air by exposing them to the air as promptly as can be done without affecting their solidity. But I do not limit 30 myself to the use of this method alone.

I claim—

1. As a new article of manufacture, an iron alloy containing the following elements in substantially the following proportions: 35 silicon over .1% to 3%; chromium .5% to 1.5%; nickel .25% to 1%; sulfur over .05% to .2%; phosphorus over .12% to 1.5%; manganese over .45% to 1%; and total carbon 1% to 4%.
- 40 2. As a new article of manufacture, an

alloy containing silicon, sulfur, phosphorus, manganese, carbon, nickel, chromium, and iron, the quantity of nickel being approximately fifty per cent. of the quantity of chromium.

3. As a new article of manufacture, an alloy containing silicon, sulfur, phosphorus, manganese, carbon, nickel, chromium, and iron, the quantity of chromium being largely 45 in excess of the quantity of nickel.

4. An alloy containing iron, silicon, manganese, carbon, nickel, and chromium, the quantity of chromium being largely in excess of the quantity of nickel.

5. An alloy containing iron, silicon, sulfur, phosphorus, manganese, carbon, nickel, and chromium, the quantity of manganese ranging from about .45% to about 1% of the total alloy.

6. An alloy containing iron, silicon, sulfur, phosphorus, manganese, carbon, nickel, and chromium, the quantity of sulfur ranging from about .05% to about .2% of the total alloy.

7. An alloy containing iron, silicon, sulfur, phosphorus, manganese, carbon, nickel, and chromium, the quantity of phosphorus ranging from about .12% to 1.5% of the total alloy.

8. As a new article of manufacture, an alloy containing silicon, sulfur, phosphorus, manganese, carbon, nickel, chromium, and iron, the quantity of chromium being in excess of the quantity of nickel.

Signed at Augusta, Georgia this 12th day 75 of February 1914.

JAMES RAMSEY SPEER.

Witnesses:

H. A. FLISCH,  
FRANK E. PETTIT.